

H. C. HUBBELL.  
STORAGE BATTERY ELECTRODE AND PROCESS OF MANUFACTURING IT.  
APPLICATION FILED JULY 17, 1911.

1,094,903.

Patented Apr. 28, 1914



Fig 1



Fig 2



Fig 3



Fig 4

WITNESSES:

Aldo S. Miller  
A. A. Tracy.

INVENTOR  
Harry C. Hubbell,  
BY  
Frank J. Gortz  
ATTORNEY

# UNITED STATES PATENT OFFICE.

HARRY CROSS HUBBELL, OF NEWARK, NEW JERSEY.

STORAGE-BATTERY ELECTRODE AND PROCESS OF MANUFACTURING IT.

1,094,903.

Specification of Letters Patent. Patented Apr. 28, 1914.

Application filed July 17, 1911. Serial No. 638,942.

*To all whom it may concern:*

Be it known that I, HARRY CROSS HUBBELL, a citizen of the United States, residing at Newark, in the county of Essex and State of New Jersey, have invented certain new and useful Improvements in Storage - Battery Electrodes and Processes of Manufacturing Them, of which the following is a specification.

10 My present invention is an improved iron storage battery electrode and a process of making same.

Referring now to the accompanying drawing: Figure 1 is a diagrammatic view, partly in section and partly in elevation, showing the gas furnace 9, the cylinder 6 which is inserted therein, said cylinder containing a plurality of the hard moist cakes 5, the vent hole 8 formed in the cylinder, and the cover 7, all hereinafter referred to; Fig. 2 is a diagrammatic sectional view, showing the plunger 11 which is utilized to coöperate with the die 12 in forming tablets 13 from the mixture 10 deposited within hopper 12', all as hereinafter referred to; Fig. 3 is a longitudinal sectional view of an electrode hereinafter described, showing in assembly the tablets 13, the conducting strip 14 and the gauze envelop 15, all hereinafter referred to; and Fig. 4 is a view similar to Fig. 3, of another type of electrode hereinafter described, showing in assembly the tablets 13, the conducting strip 14 and the gauze envelop 15, all hereinafter referred to.

35 Similar reference characters refer to similar parts throughout the several views of the drawing.

The preferred process is as follows:—I precipitate ferrous hydroxid from a solution of the sulfate with sodium hydroxid. This hydroxid in the form of a slime is immediately pumped into a filter press and washed, to clear it of sodium sulfate. Upon removal from the filter press, these hard, moist cakes 5 (these cakes being shown in Fig. 1 in illustration of a subsequent treatment thereof) of washed ferrous hydroxid are rapidly put into jars and tightly stoppered to prevent atmospheric action. The contents or part of the contents of these jars, as the said cakes 5 shown in Fig. 1, are subsequently dumped into an iron cylinder 6 provided with an air tight cover 7. A small vent hole is provided in the top of the cylinder 8. This cylinder and its contents are now slowly heated in a gas furnace 9 until

all the water is driven off in the form of steam. Then the temperature is raised until the cylinder has reached a dull red heat to effect the change of the ferrous hydroxid to the monoxid. The vent hole is then closed and the cylinder and contents cooled. This iron monoxid is then ground up with cadmium oxid in amount sufficient to equal about ten per cent. (10%) by weight of the total, and the resulting mixture 10 (Fig. 2) is then briqueted into small tablets each about  $\frac{1}{10}$ " square and  $\frac{1}{16}$ " thick. Exposure to the air makes no substantial change in the material of these tablets. To use them in an electrode, I place the tablets (shown in section in Figs. 3 and 4 and designated by the numeral 13) flat against both sides (as shown in Fig. 3) of a conducting strip 14 preferably of nickel  $1\frac{1}{4}'' \times 5''$  for a small portable battery, which permits 18 tablets to be applied to each side of the strip. I then fit the whole into a containing envelop 15 of nickel plated gauze, thus completing my double electrode for use between end-electrodes. On the other hand, each end electrode (an illustrative type of which is shown in Fig. 4) has the tablets 13 on only one side of the conducting strip 14, which then forms a non-perforated wall of the container for the tablets, the other wall consisting of the nickel plated gauze 15. The new material gives me an electrode for an alkaline storage battery that is reduced on charge and I find it to be extremely active and efficient. Further, it makes it unnecessary to incorporate conducting nickel filaments or other materials therewith to give conductivity, etc.

What I claim is:

1. The process of making the active material for a storage battery electrode which comprises precipitating ferrous hydroxid from a solution of a salt of iron, filtering and washing the precipitate, heating it without substantial exposure to the air to drive off the free water from the precipitate and then to a dull red heat to convert the hydroxid to iron monoxid, cooling without substantial exposure to the air and briquetting the oxid into tablets suitable for insertion into the pocket of the containing envelop of a storage battery electrode.

2. The process of making the active material for a storage battery electrode which comprises precipitating ferrous oxid from a solution of a salt of iron, filtering and washing the precipitate, heating it without

substantial exposure to the air to drive off the free water from the precipitate and then to a dull red heat to convert the hydroxid to iron monoxid, cooling without substantial exposure to the air, grinding the iron monoxid with a proportion of cadmium oxid, and briquetting the mixture into tablets suitable for insertion into the pocket of the containing envelop of a storage battery electrode.

3. The process of making the active material for a storage battery electrode which comprises converting precipitated ferrous hydroxid into iron monoxid by heating it without substantial exposure to the air, cooling the monoxid under the same condition and briquetting it into tablets suitable for insertion into the pocket of the containing envelop of a storage battery electrode.

4. The process of making the active material for a storage battery electrode which comprises converting precipitated ferrous hydroxid into iron monoxid by heating it without substantial exposure to the air, cooling the oxid under the same condition and applying it to the pocket of the containing envelop of a storage battery electrode.

5. The process of making the active material for a storage battery electrode which

comprises converting precipitated ferrous hydroxid into iron monoxid by heating it without substantial exposure to the air, cooling the monoxid under the same condition, mixing it with a proportion of cadmium oxid and briquetting the mixture.

6. An alkaline storage battery electrode which comprises a conducting containing envelop and active material contained therein, consisting of iron monoxid reduced from precipitated ferrous hydroxid by heat without substantial exposure to the air and cooled under the same condition.

7. An alkaline storage battery electrode which comprises a conducting containing envelop and active material contained therein, consisting of iron monoxid reduced from precipitated ferrous hydroxid by heat without substantial exposure to the air and cooled under the same condition, said active material further consisting of a proportion of admixed cadmium oxid.

In testimony whereof I affix my signature in presence of two witnesses.

HARRY CROSS HUBBELL.

Witnesses:

E. W. SOHERR, JR.  
S. S. NEWTON.

---

Copies of this patent may be obtained for five cents each, by addressing the "Commissioner of Patents.  
Washington, D. C."